

Feb. 8, 1966

CHIA-WEI CHEN  
PROCESS FOR MAKING A HEAVY FUEL OIL WITH RECYCLE  
VISBREAKING OF GAS OIL  
Filed June 20, 1962

3,234,118



INVENTOR.  
CHIA-WEI CHEN.

BY *Charles E. Boxley*

ATTORNEY

## 1

3,234,118

**PROCESS FOR MAKING A HEAVY FUEL OIL WITH  
RECYCLE VISBREAKING OF GAS OIL**  
Chia-Wei Chen, Freeport, N.Y., assignor to Foster  
Wheeler Corporation, New York, N.Y., a corpora-  
tion of New York  
Filed June 20, 1962, Ser. No. 203,993  
5 Claims. (Cl. 208—93)

This invention relates to recycle visbreaking of gas oil for the production of heavy fuel oil. A simplified recycle system and a process amenable to this system are offered.

In recycle visbreaking systems, heavy fuel oil is blended from vacuum pitch, thermal tar and a light cycle oil cut from visbroken gas oil. Thermal cracking or visbreaking produces a lower pour point temperature, a lower fluidity temperature and lower viscosity.

A conventional scheme for visbreaking gas oil cut from reduced crude involves the following steps:

(A) Heating and dividing reduced crude oil under a vacuum to produce a gas oil portion and bottoms which include vacuum pitch and thermal tar.

(B) Removing the bottoms for blending in a product heavy fuel oil.

(C) Visbreaking the gas oil portion in a thermal cracking zone.

(D) Dividing the visbroken gas oil to produce a top cut, an intermediate cut and a residue; with the top cut including gasoline and lighter materials; with the intermediate cut comprising light cycle oil; and with the residue including heavy gas oil and tar.

(E) Removing the intermediate cut for blending in the product heavy fuel oil.

(F) Dividing the residue under a vacuum to produce a gas oil portion and bottoms.

(G) Removing the bottoms for blending in the product heavy fuel oil.

(H) Recycling the portion of gas oil to the thermal cracking zone for visbreaking.

The present invention contemplates using the same vacuum flasher for Steps A and F. Toward this objective, the residue of Step D is recycled to the vacuum flasher used for Step A.

Basically this advance eliminates one vacuum flasher and often one heater. Energy balance opportunities are also presented with consequent utility savings.

These and other advantages will appear more fully from the accompanying idealized drawing of a system embodying the present invention. All of the equipment elements per se are well known to petroleum refineries and except for the novelty here indicated the process is known.

In the drawing, reduced crude oil is delivered from atmospheric unit 1 via line 2 to heater 3. From heater 3 the crude oil is passed via line 4 to vacuum flasher 6 wherein the above-mentioned Step A is completed producing gas oil which exits through line 7. The remainder of the feed constitutes bottoms and is exhausted via bottom line 8 as vacuum pitch and thermal tar. To accomplish Step B, line 8 transmits the vacuum pitch and thermal tar to product blender 9 wherein it becomes part of a heavy fuel oil product.

Step C calls for directly visbreaking the gas oil. Line 7 communicates the gas oil to thermal cracking furnace 11 wherein it is visbroken to give it a lower pour point temperature, a lower fluidity temperature and reduced viscosity. By directly it is meant, free of intermediate process steps.

Division according to Step D is performed in fractiona-

## 2

tor 12. Effluent from thermal cracking furnace 11 passes via line 13 directly to fractionator 12 wherein the visbroken gas oil is divided into a top cut which exits via line 14, an intermediate cut which exits via line 16 and residue which exits via line 17. The top cut includes gasoline and lighter materials. The intermediate cut comprises light cycle oil. The residue includes heavy gas oil and heavier materials.

Line 16 passes light cycle oil to blender 9 for Step E.

The crux of the present teaching is to use vacuum flasher 6 for both Steps A and F simultaneously. To accomplish Step F line 17 recycles residue from fractionator 12 to flasher 6 wherein additional gas oil is produced for visbreaking. Depending upon the temperature of the gas oil cut to be made in Step F, all or a portion of the residue recycled via line 17 may be passed through heater 3.

For control of recycle to vacuum flasher 6 it is often desirable to draw off a portion of the residue. Accordingly line 17 is connected to product blender 9 via line 18.

As in prior systems the additional gas oil produced in Step F is recycled to thermal cracking furnace 11. In the present system this delivery is accomplished by line 7 which also serves to deliver gas oil produced by Step A to the thermal cracking furnace.

Step F produces vacuum pitch and thermal tar in vacuum flasher 6 as did Step A. Accordingly, Step G, the passing of vacuum pitch and thermal tar to the product blender 9 is accomplished by line 8 which also accomplishes Step B.

This system is especially suitable for light crudes such as those from the Sahara Desert. These crudes tend toward instability of heavy fuel oil. A representative Sahara crude is characterized in Table I. In Table II this process is compared with a conventional two-pass visbreaking process. The upper portion of Table II presents results obtained when residue is recycled via line 17 to upstream of heater 3. The lower side of Table II relates comparable results for the same crude visbroken according to the conventional process. It should be noted that pour point temperature is lower with the present process. Also the difference between the bottom sediment and water before and after oxidation is a commercially acceptable 0.3 as compared to a woefully unstable 2.85 by the conventional process.

It will be apparent that wide changes may be made in the details of the shown embodiment without departing from the spirit of invention set forth in the claims.

50

TABLE I  
*Representative Sahara crude*

|                        |      |
|------------------------|------|
| Gravity, ° API         | 39.3 |
| 55 Viscosity, SSU, at— |      |
| 72° F.                 | 42.7 |
| 100° F.                | 39.0 |
| Pour point, ° F.       | 15   |
| 60 ASTM distillation:  | ° F. |
| IBP                    | 118  |
| 5%                     | 194  |
| 10%                    | 229  |
| 20%                    | 293  |
| 30%                    | 364  |
| 40%                    | 437  |
| 50%                    | 520  |
| 60%                    | 579  |
| 65 62%                 | 600  |

**3**  
**TABLE II**

*Heavy fuel oil production*

[With residue from fractionator recycled to vacuum flasher]

|                           | 650° F./950° F.<br>Charge<br>Vacuum<br>Gas Oil | Heavy Fuel<br>Oil From<br>First Pass<br>Operation | Product<br>Heavy Fuel<br>Oil | 5  |
|---------------------------|------------------------------------------------|---------------------------------------------------|------------------------------|----|
| Gravity, ° API            | 26.1                                           | 20.7                                              | 19.9                         | 10 |
| Viscosity, SSU, at        |                                                |                                                   |                              |    |
| 100° F.                   |                                                | 474                                               | 319                          |    |
| 150° F.                   | 73.6                                           | 120.5                                             | 101.4                        |    |
| 210° F.                   | 46.0                                           |                                                   |                              |    |
| Pour Point, ° F.          | 105                                            | 60                                                | 45                           |    |
| Stability:                |                                                |                                                   |                              |    |
| BSW before O <sub>2</sub> | 0.1                                            | 0.2                                               | 0.2                          | 15 |
| BSW after O <sub>2</sub>  | 0.4                                            | 0.35                                              | 0.5                          |    |

[With first vacuum flasher and recycle from second vacuum flasher]

|                           | Charge<br>Reduced<br>Crude | Heavy Fuel<br>Oil From<br>First Pass<br>Operation | Product<br>Heavy Fuel<br>Oil | 20 |
|---------------------------|----------------------------|---------------------------------------------------|------------------------------|----|
| Gravity, ° API            | 21.4                       | 22.4                                              | 21.3                         |    |
| Viscosity, SSU, at        |                            |                                                   |                              |    |
| 100° F.                   |                            | 250.6                                             | 180.8                        | 25 |
| 150° F.                   | 198.0                      | 89.0                                              | 70.5                         |    |
| 210° F.                   | 75.0                       |                                                   |                              |    |
| Pour Point, ° F.          | 100                        | 70                                                | 60                           |    |
| Stability:                |                            |                                                   |                              |    |
| BSW before O <sub>2</sub> | 0.7                        | 0.25                                              | 0.15                         |    |
| BSW after O <sub>2</sub>  | 0.8                        | 4.70                                              | 3.0                          |    |

5  
**4**

refining a single heating zone and a single fractionating zone,

passing atmospheric reduced crude oil serially through the single heating zone and the single fractionating zone to produce a gas oil portion and bottoms,

passing directly the gas oil portion to a thermal cracking zone for thermal cracking therein,

passing directly the thermally cracked gas oil to a fractionator zone for division to produce a residue of the thermally cracked gas oil including heavy oil and heavier materials,

recycling the residue directly to the single heating zone and the single fractionating zone for fractionation together with the atmospheric reduced crude oil,

the single fractionating zone further producing residue bottoms from the residue,

removing the bottoms and the residue bottoms together from the single fractionating zone,

blending the bottoms and residue bottoms with a light oil fraction to produce heavy fuel oil.

3. A process for producing heavy fuel oil from reduced crude oil comprising the steps of, defining a single heating zone and a single fractionating zone,

passing atmospheric reduced crude oil serially through the single heating zone and the single fractionating zone to produce a gas oil portion and bottoms,

passing directly the gas oil portion to a thermal cracking zone for thermal cracking therein,

passing directly the thermally cracked gas oil to a fractionator zone for division to produce a residue of the thermally cracked gas oil and a top cut and an intermediate cut, said top cut including gasoline and lighter materials,

said residue including heavy gas oil and heavier materials,

recycling the residue directly to the single heating zone and the single fractionating zone for fractionation together with the atmospheric reduced crude oil,

the single fractionating zone further producing residue bottoms from the residue,

removing the bottoms and the residue bottoms together from the single fractionating zone,

blending the bottoms and residue bottoms with a light oil fraction to produce heavy fuel oil.

4. The process of claim 3 with the intermediate cut comprising light cycle oil, and wherein the light oil fraction blended with the bottoms and residue bottoms comprises said intermediate cut.

5. The process of claim 4 with the fractionating zone operated under subatmospheric pressure.

**References Cited by the Examiner**

**UNITED STATES PATENTS**

|           |         |                |        |
|-----------|---------|----------------|--------|
| 2,633,449 | 3/1953  | Cheney         | 208—76 |
| 2,651,601 | 9/1953  | Taff et al.    | 208—94 |
| 2,663,675 | 12/1953 | Ewell          | 208—73 |
| 2,717,856 | 9/1955  | Ricards et al. | 208—15 |
| 3,110,663 | 11/1963 | Miller         | 208—93 |

55  
**DELBERT E. GANTZ, Primary Examiner**

65  
**ALPHONSO D. SULLIVAN, Examiner**

**H. LEVINE, Assistant Examiner**

UNITED STATES PATENT OFFICE  
CERTIFICATE OF CORRECTION

Patent No. 3,234,118

February 8, 1966

Chia-Wei Chen

It is hereby certified that error appears in the above numbered patent requiring correction and that the said Letters Patent should read as corrected below.

Column 4, line 1, for "refining" read -- defining --;  
line 10, after "heavy" insert -- gas --.

Signed and sealed this 7th day of February 1967.

(SEAL)

Attest:

ERNEST W. SWIDER

Attesting Officer

EDWARD J. BRENNER  
Commissioner of Patents